

July 1, 1947.

G. K. TEAL

PHOTOELECTROMOTIVE FORCE CELL OF THE SILICON-SILICON  
OXIDE TYPE AND METHOD OF MAKING THE SAME  
Original Filed Jan. 30, 1943 2 Sheets-Sheet 1

2,423,125

FIG. 1



FIG. 2



FIG. 3



INVENTOR  
G. K. TEAL

BY *Hugh S. Wertz*

ATTORNEY

July 1, 1947.

G. K. TEAL

2,423,125

PHOTOELECTROMOTIVE FORCE CELL OF THE SILICON-SILICON  
OXIDE TYPE AND METHOD OF MAKING THE SAME

Original Filed Jan. 30, 1943 2 Sheets-Sheet 2



FIG. 4



FIG. 5



FIG. 6



FIG. 7



FIG. 8



FIG. 9

INVENTOR  
G. K. TEAL  
BY *Hugh S. Allen*

ATTORNEY

## UNITED STATES PATENT OFFICE

2,423,125

PHOTOELECTROMOTIVE FORCE CELL OF  
THE SILICON-SILICON OXIDE TYPE AND  
METHOD OF MAKING THE SAMEGordon K. Teal, Summit, N. J., assignor to Bell  
Telephone Laboratories, Incorporated, New  
York, N. Y., a corporation of New YorkOriginal application January 30, 1943, Serial No.  
474,205. Divided and this application May 16,  
1944, Serial No. 535,798

8 Claims. (Cl. 136—89)

1

This invention relates to electro-optical devices and more specifically to photo-E. M. F. devices and to methods of making them.

This application is a division of application Serial No. 474,205, filed January 30, 1943.

A photo-E. M. F. device may be defined as a material, combination of materials or cell which when electromagnetic radiations of certain short wavelength, like those, for example, to which the eye is sensitive, are applied thereto will produce an electromotive force across its terminals, or across two portions thereof which can serve as terminals. The voltage set up between the terminals of a photo-E. M. F. device or cell when such waves are applied thereto may be used, by way of example, to control an electron beam. In describing the invention, such waves will be called "light," but this term is used in a broad sense to be inclusive also of radiations to which the eye is not sensitive.

Objects of this invention are to provide sensitive and cheap photo-E. M. F. cells and methods of making them.

In accordance with a specific embodiment of the invention, chosen by way of example for purposes of illustration, there is provided a photo-E. M. F. cell comprising a metal base, a coating comprising a mixture of silicon and a metal of higher conductivity than silicon on the base, a layer of silicon on the coating, and a layer of an oxide of silicon, such as quartz, mixed with a metallic material on said silicon layer, and a metallic member, such as a thin metallic coating, on the last-mentioned layer. In accordance with the invention, this cell, by way of example, can be formed by simultaneously evaporating silicon and a metal of higher conductivity than silicon, such as aluminum, arsenic, titanium, copper or silver, on a metal base, evaporating silicon alone on this combination or mixed layer, covering the silicon layer with quartz (silicon dioxide) and tungsten or another metal, and then applying a thin metallic coating on the quartz and metallic material. The effect of the metal of higher conductivity is to give the cell a lower internal resistance than would otherwise be obtained. Instead of simultaneous evaporation, the silicon and the metal of greater conductivity can be applied in alternate very thin layers which partially merge with each other.

Photo-E. M. F. cells or devices of the type described above can be utilized in a television electron camera tube which comprises an evacuated envelope enclosing means for generating a beam of electrons, and an apertured target for said

2

beam comprising an apertured metal screen or plate carrying on the side remote from the beam generating means a multiplicity of elemental photo-E. M. F. cells. An image of an object is projected upon the photo-E. M. F. cells and the other side of the target is scanned with the beam of electrons.

The principle of operation of this tube is as follows: The beam generating means produces a relatively high velocity beam and this is caused to scan the side of the target remote from the photo-E. M. F. cells. These cells have applied thereto light radiations from the object to be televised and there is produced across each cell a voltage proportional to the light striking the cell from a corresponding elemental area of the object. The scanning beam strikes the target plate and causes the emission of secondary electrons which pass through the apertures in the target member to a collecting electrode placed within the tube between the target and the object. The number of electrons which pass through any aperture is controlled by the voltage across the neighboring elemental photo-E. M. F. cells. The collecting electrode is connected to a signal resistor through which passes the video current, which is amplified by any suitable amplifier.

Obviously, the photo-E. M. F. cells or devices in accordance with the invention are not limited to use in electron camera tubes as they may have a wide variety of other uses for which photo-E. M. F. cells are, in general, adapted.

The invention will be more readily understood by referring to the following description taken in connection with the accompanying drawing forming a part thereof, in which:

Fig. 1 is a schematic representation of a cathode ray tube and certain of its associated circuits, the tube employing photo-E. M. F. cells in accordance with the invention;

Fig. 2 is a schematic view showing, in greatly enlarged form, a portion of the target and of the electron collecting electrode of the tube shown in Fig. 1;

Fig. 3 is an enlarged front view of a portion of the target; and

Figs. 4 to 9, inclusive, are diagrammatic representations to aid in explaining the invention.

Referring more particularly to the drawings, Fig. 1 shows, by way of example to illustrate the invention, a cathode ray television transmitter tube 10 employing a two-sided mosaic target 11 containing photo-E. M. F. elements. The tube 10 comprises an evacuated container 12 enclosing the mosaic target 11, an electron gun 13 for gen-

erating, focusing and accelerating a beam of high velocity electrons towards this target, a secondary electron collecting electrode 14 on the side of the target 11 remote from the electron gun 13, and two sets of electrostatic deflecting plates 15 and 16 for causing the beam of electrons to scan every elemental area in turn of a field of view on the mosaic target 11. Radiations from an object or field of view O are applied to the side of the mosaic target 11 remote from the electron gun by means of any suitable optical system represented schematically by the lens 17.

The electron gun 13 preferably comprises a cathode 20, a control electrode or member 21, a first anode member 22, and a second and final anode member comprising a cylindrical member 23 and a coating 24 of conducting material on the inside walls of the envelope 12 extending from the region of the cylinder 23 to the region of the mosaic target. The collecting electrode 14 for the secondary electrons emitted from the target 11 when it is struck by the beam of high velocity electrons preferably consists of mesh material or, if desired, it may consist of a ring of metallic material.

The control electrode 21 is placed at any suitable negative potential with respect to the potential of the cathode 20 by means of an adjustable source 38; and the first anode 22 and the final anode 23, 24 are placed at appropriate positive potentials with respect to the cathode 20 by means of the source 31 and the source 32. As an example, the final anode 23, 24 can be about 1,000 volts positive with respect to the cathode and the first anode 22 can be 300 volts positive with respect to the cathode. Any suitable source 35 can be utilized to heat the cathode 20. The negative terminal of the source 31 is connected to the cathode 20 and the positive terminal thereof is connected to the first anode 22, while the negative terminal of the source 32 is connected to the positive terminal of the source 31 and the positive terminal of source 32 is connected to the second anode 23, 24. Preferably the positive terminal of the source 32 is connected to ground through a source 37 which is used to make the apertured plate 50 (see Fig. 2) of the target 11 positive with respect to the final anode of the electron gun for a purpose which will be pointed out hereinbelow. The voltage of this source 37 can be, for example, 20 to 50 volts. The apertured plate 50 is connected to ground and is also connected through a source 33 and a signal resistor 34 to the collecting electrode 14. Any suitable amplifier 36 is connected to the signal resistor 34 and is in turn connected to the other elements of the television transmitter circuit which prepare the video current for transmission to the receiving station. The potentials applied to the various electrode members and their configuration and shape are such that a beam of focussed high velocity electrons strikes the target 11 and this beam is deflected over a suitable field thereon by means of appropriate potentials applied to the deflecting plates 15 and 16 by electrostatic sweep circuits (not shown) to produce secondary electrons, the action of which will be considered more fully below. As examples of satisfactory sweep circuits, reference may be made to Patent No. 2,178,464, dated October 31, 1939, to M. W. Baldwin, Jr., which discloses balanced electrostatic sweep circuits suitable for this purpose. Connections can be made from the balanced sweep circuits to the pairs of plates 15 and 16 by means of coupling condensers 40, 41 and 42, 75

43, respectively, of about one microfarad capacity each. Coupling resistances 44 and 45 of the order of many megohms each are respectively connected across the pairs of plates 15 and 16. The mid-points of the resistances 44 and 45 are connected to the positive terminal of the source 32 so that the average of the potentials of the deflecting plates does not deviate more than slightly from the potential of the anode 23, 24. This relationship is maintained to avoid changes in the sensitivity of the deflecting system and the consequent distortion of the image which would otherwise result. For more complete descriptions of the advantages of balanced sweep circuits for use with cathode ray television tubes, reference is made to the above-mentioned Baldwin patent and also to Patent 2,209,199, issued July 23, 1940, to Frank Gray.

Reference will now be made to Figs. 2 and 3 which are enlarged schematic views of a preferred form of mosaic target 11. Fig. 2 is a schematic side view, in cross section, of a portion of the target 11, while Fig. 3 is an enlarged showing of a portion of the target 11, viewed from the right in Fig. 2, to show the general relationship of the apertures 52 in the target and the photo-E. M. F. cells 51 thereof. Certain dimensions in Figs. 2 and 3 have been exaggerated at the expense of others in order to more clearly show the screen structure. The mosaic target 11 preferably comprises an apertured plate 50 of any suitable material, such as nickel, carrying thereon on the side remote from the beam generating means a multiplicity of photo-E. M. F. cell elements 51, each aperture 52 in the plate being effectively surrounded by cell elements. Each of the elements 51 can comprise, for example, a small copper-oxide photo-E. M. F. cell which cell, as is well known in the art, generally comprises a layer of copper, a semiconducting layer of cuprous oxide thereon treated by means well-known in the art to produce on the semiconducting layer a blocking layer, and a thin semitransparent conducting element such as silver or gold covering the blocking layer. In the preferred embodiment, however, the elements are of the silicon-silicon oxide type to be described more fully below.

Reference will now be made to Figs. 4 to 8, inclusive, which illustrate a method of making a suitable target structure 11. Figs. 4 to 8 are schematic views showing a number of small photo-E. M. F. cells on a target (but not showing all that would be normally shown by a cross-sectional view in order to simplify the drawings). The relative dimensions of Figs. 4 to 8, inclusive, are, of course, not exactly correct, the only purpose of these figures being to illustrate the process. A satisfactory method of making the target structure 11 of the tube and utilizing copper-copper oxide type cells is as follows: A perforated screen or plate 50 of nickel or any other suitable metal, made by any well-known commercial process, has a greased or waxed surface 60 thereof insullated with a suitable protective covering material, such as asphaltum particles small in comparison with the diameter of holes 52 in the screen. The screen 50 has, for example, 100 to 200 or more apertures per inch. It is slightly warmed to cause the asphaltum deposit to flow and produce a multiplicity of dot-like elements 62 fairly evenly distributed over the surface of the plate as shown in Fig. 4. The back of the plate is then covered with an asphaltum covering 63 (see Fig. 5) which can be done without the as-

phaltum going completely through to the insulfated side by pouring asphaltum varnish of the correct consistency on the back of the screen and allowing it to dry. A silver or other suitable metallic mask 64 is then plated on the unprotected areas of the plate 50, the greasy or waxy coating 60 making it possible for the silver to be later stripped off. This is shown in Fig. 6. Due to the fact that the grease film is very thin, there are various minute openings therein and thus the silver reaches through these openings to the metal layer underneath and attaches itself to the metal layer. It is not as firm a coating, however, as would be the case if the grease film were not there and hence the silver can be easily stripped off at the proper time in the method. The grease can be applied either before or after the asphalt, but preferably it is applied first. All the asphaltum is then dissolved in benzene. A copper film 65 is then deposited on the plated side of the member 50 by evaporation. The appearance of the target after these last two steps is schematically represented by Fig. 7. The copper is deposited directly on the metal since all the grease and asphaltum has been dissolved by the benzene. Hence the copper is firmly adherent to the metal electrode whereas the silver, being not so firmly adherent, can be stripped off without the copper being stripped off with it. The silver mask or screen 64 is then carefully stripped away leaving small dots 65 of copper where the asphaltum dots had formerly been. The silver can be stripped away, for example, by grasping one end of the mask by a suitable holding tool and very carefully lifting the mask while holding the target firmly until the whole mask is stripped from the target. The copper dots are then oxidized by any suitable means (such as by heating the entire target in oxygen) and the oxide surfaces 66 treated by electron or ion bombardment to produce a blocking layer 67 for each small cell. A very thin semitransparent film 68 of gold or other suitable conducting material is evaporated onto the small cell surfaces. The gold film is not confined to the cell surfaces nor need it be since it is so thin that its resistance is very high laterally of the target. By this process there is produced a number of small sandwich-type photo-E. M. F. cells distributed at random over the screen. If desired, the copper dots 65 can be oxidized, treated, and the semitransparent film 68 evaporated thereon before the silver mask 64 is stripped off. These cells are of the type known as a "front wall" cell. In these cells, a negative potential with respect to the plate 50 is acquired by the semitransparent metal layer 68 when light radiations are applied to the cells from the object O. If desired, the cells can be produced by any suitable process which produces a "back wall" type of cell but cells of this latter type are generally not so sensitive as those of the "front wall" type. If the cells 51 are of the "back wall" type, the semitransparent metal layer becomes positive with respect to the plate 50 when light radiations are applied to the cells. The arrangement in accordance with this invention is operable with either type of cell and, moreover, is not limited to the use of the copper oxide type or of the silicon-silicon oxide type now to be described.

If desired, the surface of the target nearer the beam can be treated in a manner to enhance the production of low velocity secondary electrons by evaporating a thin layer of a suitable metal, such as magnesium, on this surface and then wholly or partially oxidizing this metal layer.

When the cells are of the silicon-silicon oxide type, they can be made as follows: First, silicon (instead of copper) is deposited on the silver-plated side of the mosaic after the asphaltum has been dissolved. A more to be preferred method is to deposit the "silicon" in two layers, one by simultaneous evaporation of silicon and a metal of higher conductivity than silicon, such as aluminum, arsenic, titanium, copper or silver, and the second by evaporation of silicon alone. The effect of the metal of higher conductivity is to give the cell a lower internal resistance than would otherwise be obtained. The silicon (or silicon and the conducting metal) layer is then covered by evaporation of quartz (silicon dioxide) or another suitable insulator with tungsten or another suitable element such as silicon, molybdenum, or tantalum. The evaporation can be effected either simultaneously or in alternate thin layers as the layers are very thin and not very smooth, thus permitting one to partially merge with the other. Finally, a thin semi-transparent film of gold, silver or other suitable conducting material is evaporated onto the small cell surfaces and the silver mask and the films on it are stripped away, leaving small sandwich-type silicon oxide photo-E. M. F. cells distributed at random over the screen. Such photo-E. M. F. cells, greatly enlarged, are shown in Fig 9. The silicon-silicon oxide cell described above is of particular advantage in the camera tube in accordance with this invention because of its low impedance. Because of this, electrons which fall back on the surface of the target remote from the beam do not charge this surface.

The operation of the arrangement shown in Fig. 1 is as follows, reference also being made to Figs. 2 and 3. Radiations from an object or field of view are projected upon the right-hand side of the mosaic target 11 by means of the lens system 17. A high velocity beam of electrons generated by the electron gun 13 is deflected over a field of the mosaic target 11 corresponding to the area covered by the radiations from the object by means of deflecting potentials applied to the deflecting plates 15 and 16. As shown in Fig. 2, the cathode ray beam is generally of such size that it covers several apertures 52 and the spaces between them. It will be appreciated that the lines indicating the beams are not accurately representative of the electron paths since obviously the electric fields adjacent the apertures of the member 50 are not uniform and produce a certain amount of convergence or divergence. When the primary beam strikes the metal member 50, secondary electrons are given off and these secondary electrons (mixed with some primary electrons which are not shown in the drawing in order to simplify it) pass through the aperture or apertures 52 adjacent the scanning spot to the collecting electrode 14. The source 37 places the plate 50 at a positive potential of from 20 to 50 volts with respect to the electrode 24 to allow only electrons originating next to an aperture to go through it, or, in other words, a field is established which discourages secondary electrons from traveling from one point of the target to another. The number of secondary electrons which pass through any particular aperture 52 is dependent upon the potential generated across the adjacent individual photo-E. M. F. cells 51 by the radiations applied thereto from the corresponding elemental area of the object. The action of the photo-E. M. F. cells 51 is somewhat analogous to that of a grid in a triode. This volt-

age between the semitransparent metal member 68 and the metal screen member 50 varies the number of secondary electrons which pass through the corresponding aperture 52. This voltage has practically no effect on the primary electrons but as the number of them passing through the target 11 in a given time interval remains substantially constant, these electrons contribute only to the "average" or background current flowing through the resistor 34 and do not affect the signal current. Moreover, secondary electrons emitted from the plate 50 which do not go through the apertures 52 and are picked up by the plate 50 do not introduce distortion in the signal current as the plate 50 is maintained at a fixed potential. If any secondary electrons fall back on the side of the cells 51 remote from the electron beam, they are immediately conducted to the plate 50 as the resistance of the cells is relatively low. Unlike the storage type of camera tube using photoemissive elements wherein each photoemissive element must be discharged once per cycle, the photo-E. M. F. cells 51 can have the potential thereacross varied at will (by the change in light) and need not have this potential brought to zero once every scanning cycle. The variable current passing through the resistor 34 constitutes the video signal current and this current is amplified by the amplifier 36 in a manner well known in the art. The video current is then caused to modulate a carrier for transmission to a distant station by means well known.

Various modifications can be made in the embodiment described above without departing from the spirit of the invention, the scope of which is indicated by the appended claims.

What is claimed is:

1. A photo-E. M. F. cell comprising a metal base, a coating comprising a mixture of silicon and a metal of higher conductivity than silicon on said base, a layer of silicon on said coating, a layer of quartz mixed with a metallic material on said silicon layer, and a metallic member in contact with said last mentioned layer.

2. A photo-E. M. F. cell comprising a metal base, a coating comprising a mixture of silicon and a metal of higher conductivity than silicon on said base, a layer of silicon on said coating, a layer of an oxide of silicon mixed with a metallic material on said silicon layer, and a metallic member in contact with said last mentioned layer.

3. A method of making a photo-E. M. F. cell comprising the steps of simultaneously evaporating silicon and a metal of higher conductivity on a metal base to form a composite coating of the two materials thereon, forming a layer of silicon on said coating, forming a layer of an oxide of silicon on said silicon layer, and applying a thin,

semi-transparent metallic coating on said last mentioned layer.

4. A photo-E. M. F. cell comprising a metal base, a coating comprising a mixture of silicon and one of the group consisting of aluminum, arsenic, titanium, copper and silver on said base, a layer of silicon on said coating, a layer of an oxide of silicon mixed with an element from the group consisting of tungsten, silicon, molybdenum and tantalum on said silicon layer, and a metallic member in contact with said last mentioned layer.

5. A method of making a photo-E. M. F. cell comprising the steps of simultaneously evaporating silicon and a metal of higher conductivity on a metal base to form a composite coating of the two materials thereon, forming a layer of silicon on said coating, forming a layer of an oxide of silicon on said silicon layer, and applying a thin, semi-transparent metallic coating on said oxide layer.

6. A method of making a photo-E. M. F. cell comprising the steps of simultaneously evaporating a coating of silicon and a metal of higher conductivity on a metal base, forming a layer of silicon on said coating, applying quartz and a metallic material simultaneously to said silicon layer, and applying a thin, semi-transparent metallic coating on said quartz and metallic material.

7. A method of making a photo-E. M. F. cell comprising the steps of simultaneously evaporating a coating of silicon and a metal of higher conductivity on a metal base, forming a layer of silicon on said coating, applying alternate thin layers of quartz and metallic material to said silicon layer, and applying a thin, semi-transparent metallic coating on said oxide layer.

8. A method of making a photo-E. M. F. cell comprising the steps of evaporating a coating of silicon and tungsten on a metal base, forming a layer of silicon on said coating, forming a layer of an oxide of silicon on said silicon layer, and applying a thin, semi-transparent metallic coating on said oxide layer.

45 GORDON K. TEAL.

#### REFERENCES CITED

The following references are of record in the file of this patent:

#### UNITED STATES PATENTS

| Number     | Name    | Date          |
|------------|---------|---------------|
| Re. 22,052 | Geisler | Mar. 24, 1942 |
| 2,234,696  | Hewlett | Mar. 11, 1941 |

#### 55 FOREIGN PATENTS

| Number  | Country       | Date         |
|---------|---------------|--------------|
| 314,838 | Great Britain | July 3, 1929 |